



US008609599B2

(12) **United States Patent**  
**Hartley**

(10) **Patent No.:** **US 8,609,599 B2**  
(45) **Date of Patent:** **Dec. 17, 2013**

(54) **MARINE ENGINE LUBRICATION**

(75) Inventor: **Joseph P. Hartley**, Oxford (GB)

(73) Assignee: **Infineum International Limited** (GB)

(\*) Notice: Subject to any disclaimer, the term of this patent is extended or adjusted under 35 U.S.C. 154(b) by 0 days.

(21) Appl. No.: **13/277,331**

(22) Filed: **Oct. 20, 2011**

(65) **Prior Publication Data**

US 2012/0103303 A1 May 3, 2012

(30) **Foreign Application Priority Data**

Oct. 28, 2010 (EP) ..... 10189226

(51) **Int. Cl.**

**C09K 15/08** (2006.01)  
**C10M 159/22** (2006.01)  
**F02B 1/12** (2006.01)

(52) **U.S. Cl.**

USPC ..... **508/584**; 508/460; 123/27 R

(58) **Field of Classification Search**

USPC ..... 123/27 R; 508/584, 460  
See application file for complete search history.

(56) **References Cited**

U.S. PATENT DOCUMENTS

2,476,696 A \* 7/1949 Caplan et al. ..... 508/580  
2012/0028522 A1 \* 2/2012 Garner et al. ..... 440/88 L

OTHER PUBLICATIONS

Moreira et al., Stabilization of Asphaltenes by Phenolic Compounds Extracted from Cashew-Nut Shell Liquid, Apr. 19, 1999, Journal of Applied Polymer Science, vol. 73, Issue 1, pp. 29-34.\*

\* cited by examiner

*Primary Examiner* — Cephia D Toomer

*Assistant Examiner* — Vishal Vasisth

(57) **ABSTRACT**

Trunk piston marine engine lubrication, when the engine is fueled by heavy fuel oil, is effected by a composition comprising a major amount of an oil of lubricating viscosity and a minor amount of one or more phenolic compounds comprising distilled cashew nut shell liquid or hydrogenated distilled cashew nut shell liquid. Asphaltene precipitation in the lubricant, caused by the presence of contaminant heavy fuel oil, is prevented or inhibited.

**10 Claims, No Drawings**

## MARINE ENGINE LUBRICATION

## FIELD OF THE INVENTION

This invention relates to a trunk piston marine engine lubricating composition for a medium-speed four-stroke compression-ignited (diesel) marine engine and lubrication of such an engine.

## BACKGROUND OF THE INVENTION

Marine trunk piston engines generally use Heavy Fuel Oil ('HFO') for offshore running. Heavy Fuel Oil is the heaviest fraction of petroleum distillate and comprises a complex mixture of molecules including up to 15% of asphaltenes, defined as the fraction of petroleum distillate that is insoluble in an excess of aliphatic hydrocarbon (e.g. heptane) but which is soluble in aromatic solvents (e.g. toluene). Asphaltenes can enter the engine lubricant as contaminants either via the cylinder or the fuel pumps and injectors, and asphaltene precipitation can then occur, manifested in 'black paint' or 'black sludge' in the engine. The presence of such carbonaceous deposits on a piston surface can act as an insulating layer which can result in the formation of cracks that then propagate through the piston. If a crack travels through the piston, hot combustion gases can enter the crankcase, possibly resulting in a crankcase explosion.

It is therefore highly desirable that trunk piston engine oils ('TPEO's) prevent or inhibit asphaltene precipitation. The prior art describes ways of doing this.

WO 96/26995 discloses the use of a hydrocarbyl-substituted phenol to reduce 'black paint' in a diesel engine.

Cashew nut shells contain approximately 40% phenolic compounds. They are readily available worldwide and potentially constitute a low-cost, widely-available and renewable raw material for phenols. "Stabilization of Asphaltenes by Phenolic Compounds Extracted from Cashew-Nut Shell Liquid" Moreira, Lucas and Gonzalez, Journal of Applied Polymer Science, Vol. 73, 29-34 (1999) (herein "Moreira et al") describes the use of phenolic compounds extracted from cashew nut shell liquid (herein "CNSL") for the stabilisation of asphaltenes, but in crude oil. Specifically, Moreira et al show that technical CNSL (obtained by roasting the shells to extract liquid) and cardanol (obtained by distilling technical CNSL) are both effective at stabilizing asphaltenes in toluene/heptane mixtures.

Moreira et al do not, however, address the problem of asphaltene precipitation in TPEO's, which have a different properties compared with crude oil. They remark that technical CNSL and cardanol contain phenolic compounds with long linear alkyl chains containing 15 carbon atoms with variable unsaturation degrees, meta-substituted in the aromatic ring. They further remark that side-chain unsaturation seems an attractive possibility to improve the efficiency of phenolic compounds to disperse asphaltic dispersions.

"Chemistry and Technology of Lubricants" (Second Edition) edited by Mortier and Orszulik discusses the properties and formulation of marine lubricants (paragraph 10.6) and summarises typical properties of the three types of marine diesel engine lubricants, i.e. system oil, cylinder oil and TPEO. It notes that the three types of oils have quite different performance requirements and summarises these also. Paragraph 10.9 discusses TPEO's in more detail such as issues arising from their use in engines operating on HFO.

## SUMMARY OF THE INVENTION

It is now found that technical CNSL, used in combination with salicylate detergents, is not effective to stabilize asphalt-

enes in TPEO's, but surprisingly, that cardanol is effective and that analogous phenols in which the long linear alkyl chains are saturated, (i.e. not mentioned by Moreira et al) are even more effective.

5 A first aspect of the invention is a trunk piston marine engine lubricating oil composition for improving asphaltene handling in use thereof in operation of the engine when fuelled by a heavy fuel oil, which composition comprises or is made by admixing an oil of lubricating viscosity, in a major 10 amount, preferably containing 50 mass % or more of base-stock containing greater than or equal to 90% saturates and less than or equal to 0.03% sulphur or a mixture thereof, and, in a minor amount:

(A) one or more oil-soluble phenolic compounds, comprising distilled cashew nut shell liquid or hydrogenated distilled cashew nut shell liquid, provided that, in the absence of a hydroxybenzoate detergent, the mass percentage of the phenolic compound is 4 or 5 or 6 or 7 or more.

15 20 A second aspect of the invention is the use of component (A) as defined in the first aspect of the invention, in a minor amount, in a trunk piston marine lubricating oil composition for a medium-speed compression-ignited marine engine to improve asphaltene handling during operation of the engine, fueled by a heavy fuel oil, and its lubrication by the composition.

25 30 A third aspect of the invention is a method of dispersing asphaltenes in a trunk piston marine lubricating oil composition during its lubrication of surfaces of the combustion chamber of a marine-speed compression-ignited marine engine and operation of the engine, which method comprises

35 (i) providing a composition as defined in the first aspect of the invention;  
(ii) providing the composition in the combustion chamber;  
(iii) providing heavy fuel oil in the combustion chamber; and  
(iv) combusting the heavy fuel oil in the combustion chamber.

40 45 A fourth aspect of the invention is a method of operating a trunk piston engine medium-speed compression-ignited marine engine comprising

(i) fueling the engine with a heavy fuel oil; and  
(ii) lubricating the crankcase of the engine with a composition as defined in the first aspect of the invention.

In this specification, the following words and expressions, if and when used, have the meanings ascribed below:

"active ingredients" or "(a.i.)" refers to additive material that is not diluent or solvent;

"comprising" or any cognate word specifies the presence of stated features, steps, or integers or components, but does not preclude the presence or addition of one or more other features, steps, integers, components or groups thereof; the expressions "consists of" or "consists essentially of" or cognates may be embraced within "comprises" or cognates, wherein "consists essentially of" permits inclusion of substances not materially affecting the characteristics of the composition to which it applies;

"major amount" means in excess of 50 mass % of a composition;

"minor amount" means less than 50 mass % of a composition;

"TBN" means total base number as measured by ASTM D2896.

60 65 Furthermore in this specification:

"calcium content" is as measured by ASTM 4951;

"phosphorus content" is as measured by ASTM D5185;

"sulphated ash content" is as measured by ASTM D874; "sulphur content" is as measured by ASTM D2622; "KV100" means kinematic viscosity at 100° C. as measured by ASTM D445.

Also, it will be understood that various components used, essential as well as optimal and customary, may react under conditions of formulation, storage or use and that the invention also provides the product obtainable or obtained as a result of any such reaction.

Further, it is understood that any upper and lower quantity, range and ratio limits set forth herein may be independently combined.

#### DETAILED DESCRIPTION OF THE INVENTION

The features of the invention will now be discussed in more detail below.

##### Oil of Lubricating Viscosity

The lubricating oils may range in viscosity from light distillate mineral oils to heavy lubricating oils. Generally, the viscosity of the oil ranges from 2 to 40 mm<sup>2</sup>/sec, as measured at 100° C.

Natural oils include animal oils and vegetable oils (e.g., caster oil, lard oil); liquid petroleum oils and hydrorefined, solvent-treated or acid-treated mineral oils of the paraffinic, naphthenic and mixed paraffinic-naphthenic types. Oils of lubricating viscosity derived from coal or shale also serve as useful base oils.

Synthetic lubricating oils include hydrocarbon oils and halo-substituted hydrocarbon oils such as polymerized and interpolymerized olefins (e.g., polybutylenes, polypropylenes, propylene-isobutylene copolymers, chlorinated polybutylenes, poly(1-hexenes), poly(1-octenes), poly(1-decenes)); alkybenzenes (e.g., dodecylbenzenes, tetradecylbenzenes, dinonylbenzenes, di(2-ethylhexyl)benzenes); polyphenyls (e.g., biphenyls, terphenyls, alkylated polyphenols); and alkylated diphenyl ethers and alkylated diphenyl sulphides and derivative, analogs and homologs thereof.

Alkylene oxide polymers and interpolymers and derivatives thereof where the terminal hydroxyl groups have been modified by esterification, etherification, etc., constitute another class of known synthetic lubricating oils. These are exemplified by polyoxyalkylene polymers prepared by polymerization of ethylene oxide or propylene oxide, and the alkyl and aryl ethers of polyoxyalkylene polymers (e.g., methyl-polyiso-propylene glycol ether having a molecular weight of 1000 or diphenyl ether of poly-ethylene glycol having a molecular weight of 1000 to 1500); and mono- and polycarboxylic esters thereof, for example, the acetic acid esters, mixed C<sub>3</sub>-C<sub>8</sub> fatty acid esters and C<sub>13</sub> Oxo acid diester of tetraethylene glycol.

Another suitable class of synthetic lubricating oils comprises the esters of dicarboxylic acids (e.g., phthalic acid, succinic acid, alkyl succinic acids and alkenyl succinic acids, maleic acid, azelaic acid, suberic acid, sebasic acid, fumaric acid, adipic acid, linoleic acid dimer, malonic acid, alkylmalonic acids, alkenyl malonic acids) with a variety of alcohols (e.g., butyl alcohol, hexyl alcohol, dodecyl alcohol, 2-ethylhexyl alcohol, ethylene glycol, diethylene glycol monoether, propylene glycol). Specific examples of such esters includes dibutyl adipate, di(2-ethylhexyl) sebacate, di-n-hexyl fumarate, diethyl sebacate, diisooctyl azelate, diisodecyl azelate, diethyl phthalate, didecyl phthalate, dieicosyl sebacate, the 2-ethylhexyl diester of linoleic acid dimer, and the complex

ester formed by reacting one mole of sebacic acid with two moles of tetraethylene glycol and two moles of 2-ethylhexanoic acid.

Esters useful as synthetic oils also include those made from C<sub>5</sub> to C<sub>12</sub> monocarboxylic acids and polyols and polyol esters such as neopentyl glycol, trimethylolpropane, pentaerythritol, dipentaerythritol and tripentaerythritol.

Silicon-based oils such as the polyalkyl-, polyaryl-, polyalkoxy- or polyaryloxysilicone oils and silicate oils comprise another useful class of synthetic lubricants; such oils include tetraethyl silicate, tetraisopropyl silicate, tetra-(2-ethylhexyl) silicate, tetra-(4-methyl-2-ethylhexyl) silicate, tetra-(p-tert-butyl-phenyl) silicate, hexa-(4-methyl-2-ethylhexyl) disiloxane, poly(methyl)siloxanes and poly(methylphenyl) siloxanes. Other synthetic lubricating oils include liquid esters of phosphorous-containing acids (e.g., tricresyl phosphate, trioctyl phosphate, diethyl ester of decylphosphonic acid) and polymeric tetrahydrofurans.

Unrefined, refined and re-refined oils can be used in lubricants of the present invention. Unrefined oils are those obtained directly from a natural or synthetic source without further purification treatment. For example, a shale oil obtained directly from retorting operations; petroleum oil obtained directly from distillation; or ester oil obtained directly from an esterification and used without further treatment would be an unrefined oil. Refined oils are similar to unrefined oils except that the oil is further treated in one or more purification steps to improve one or more properties. Many such purification techniques, such as distillation, solvent extraction, acid or base extraction, filtration and percolation are known to those skilled in the art. Re-refined oils are obtained by processes similar to those used to provide refined oils but begin with oil that has already been used in service. Such re-refined oils are also known as reclaimed or reprocessed oils and are often subjected to additional processing using techniques for removing spent additives and oil breakdown products.

Definitions for the base stocks and base oils in this invention are the same as those found in the American Petroleum Institute (API) publication "Engine Oil Licensing and Certification System", Industry Services Department, Fourteenth Edition, December 1996, Addendum 1, December 1998. Said publication categorizes base stocks as follows:

- a) Group I base stocks contain less than 90 percent saturates and/or greater than 0.03 percent sulphur and have a viscosity index greater than or equal to 80 and less than 120 using the test methods specified in Table E-1.
- b) Group II base stocks contain greater than or equal to 90 percent saturates and less than or equal to 0.03 percent sulphur and have a viscosity index greater than or equal to 80 and less than 120 using the test methods specified in Table E-1.
- c) Group III base stocks contain greater than or equal to 90 percent saturates and less than or equal to 0.03 percent sulphur and have a viscosity index greater than or equal to 120 using the test methods specified in Table E-1.
- d) Group IV base stocks are polyalphaolefins (PAO).
- e) Group V base stocks include all other base stocks not included in Group I, II, III, or IV.

Analytical Methods for Base Stock are tabulated below:

| PROPERTY        | TEST METHOD |
|-----------------|-------------|
| Saturates       | ASTM D 2007 |
| Viscosity Index | ASTM D 2270 |

| PROPERTY | TEST METHOD |
|----------|-------------|
| Sulphur  | ASTM D 2622 |
|          | ASTM D 4294 |
|          | ASTM D 4927 |
|          | ASTM D 3120 |

As stated, the oil of lubricating viscosity preferably contains 50 mass % or more of basestock containing greater than or equal to 90% saturates and less than or equal to 0.03% sulphur or a mixture thereof. It may contain 50 mass % or more of a Group II basestock. Preferably, it contains 60, such as 70, 80 or 90, mass % or more of a Group II basestock. The oil of lubricating viscosity may be substantially all Group II basestock. Such oils are preferred because the above-mentioned problem of asphaltene precipitation is more acute at higher basestock saturate levels.

#### Phenolic Compound (A)

A characteristic structural feature of the phenolic compounds used in the invention is meta hydrocarbyl-substitution of the aromatic ring where the substituent is attached to the ring at its first (C1) carbon atom. This structural feature is not available by chemical alkyl phenol synthesis such as the Friedel-Crafts reaction of phenol with olefins. The latter typically gives mixtures of ortho and para alkyl phenols (but only around 1% of meta alkyl phenols), and where attachment of the alkyl group to the aromatic ring is at the second (C2) or higher carbon atom.

Cardanol, the product obtained by distilling technical CNSL, typically contains 3-pentadecylphenol (3%); 3-(8-pentadecenyl) phenol (34-36%); 3-(8,11-pentadecadienyl) phenol (21-22%); and 3-(8,11,14-pentadecatrienyl) phenol (40-41%), plus a small amount of 5-(pentadecyl) resorcinol (c. 10%), also referred to as cardol. Technical CNSL contains mainly cardanol plus some polymerized material. Cardanol may therefore be expressed as containing significant amounts of meta-linear hydrocarbyl substituted phenol, where the hydrocarbyl group has the formula  $C_{15}H_{25-31}$  and is attached to the aromatic ring at its first carbon atom (C1).

Thus, cardanol contains significant quantities of material having long linear unsaturated side chains and only small quantities of material with long linear saturated side chains. The present invention employs, as an additive, cardanol or, most preferably, material where a major proportion, preferably all of the phenol, contains material with long linear saturated side chains. Such latter material is obtainable by hydrogenating cardanol; a preferred example is 3-(pentadecyl) phenol, where the pentadecyl group is linear and is attached to the aromatic ring at its first carbon atom. It may constitute 50 or more, 60 or more, 70 or more, 80 or more, or 90 or more, mass % of additive compound (A). It may contain small quantities of 5-(pentadecyl) resorcinol. The invention does not include technical CNSL, which is found to be ineffective as an asphaltene dispersant.

#### Other Additives

#### Overbased Metal Detergent (B)

A metal detergent is an additive based on so-called metal "soaps", that is metal salts of acidic organic compounds, sometimes referred to as surfactants. They generally comprise a polar head with a long hydrophobic tail. Overbased metal detergents, which comprise neutralized metal detergents as the outer layer of a metal base (e.g. carbonate) micelle, may be provided by including large amounts of metal base by reacting an excess of a metal base, such as an oxide or hydroxide, with an acidic gas such as carbon dioxide.

In the present invention, overbased metal detergents such as overbased metal hydrocarbyl-substituted hydroxybenzoate, preferably hydrocarbyl-substituted salicylate, detergents may be used in minor amounts in combination with phenolic compounds (A). Salicylate detergents may be particularly useful in this respect.

"Hydrocarbyl" means a group or radical that contains carbon and hydrogen atoms and that is bonded to the remainder of the molecule via a carbon atom. It may contain hetero atoms, i.e. atoms other than carbon and hydrogen, provided they do not alter the essentially hydrocarbon nature and characteristics of the group. As examples of hydrocarbyl, there may be mentioned alkyl and alkenyl. The overbased metal hydrocarbyl-substituted hydroxybenzoate typically has the structure shown:



wherein R is a linear or branched aliphatic hydrocarbyl group, and more preferably an alkyl group, including straight- or branched-chain alkyl groups. There may be more than one R group attached to the benzene ring. M is an alkali metal (e.g. lithium, sodium or potassium) or alkaline earth metal (e.g. calcium, magnesium, barium or strontium). Calcium or magnesium is preferred; calcium is especially preferred. The COOM group can be in the ortho, meta or para position with respect to the hydroxyl group; the ortho position is preferred. The R group can be in the ortho, meta or para position with respect to the hydroxyl group. When M is divalent, it represents "half" an atom in the above formula.

Hydroxybenzoic acids are typically prepared by the carboxylation, by the Kolbe-Schmitt process, of phenoxides, and in that case, will generally be obtained (normally in a diluent) in admixture with uncarboxylated phenol. Hydroxybenzoic acids may be non-sulphurized or sulphurized, and may be chemically modified and/or contain additional substituents. Processes for sulphurizing a hydrocarbyl-substituted hydroxybenzoic acid are well known to those skilled in the art, and are described, for example, in US 2007/0027057.

In hydrocarbyl-substituted hydroxybenzoic acids, the hydrocarbyl group is preferably alkyl (including straight- or branched-chain alkyl groups), and the alkyl groups advantageously contain 5 to 100, preferably 9 to 30, especially 14 to 24, carbon atoms.

The term "overbased" is generally used to describe metal detergents in which the ratio of the number of equivalents of the metal moiety to the number of equivalents of the acid moiety is greater than one. The term 'low-based' is used to describe metal detergents in which the equivalent ratio of metal moiety to acid moiety is greater than 1, and up to about 2.

By an "overbased calcium salt of surfactants" is meant an overbased detergent in which the metal cations of the oil-insoluble metal salt are essentially calcium cations. Small amounts of other cations may be present in the oil-insoluble metal salt, but typically at least 80, more typically at least 90, for example at least 95, mole % of the cations in the oil-insoluble metal salt, are calcium ions. Cations other than calcium may be derived, for example, from the use in the manufacture of the overbased detergent of a surfactant salt in

which the cation is a metal other than calcium. Preferably, the metal salt of the surfactant is also calcium.

Carbonated overbased metal detergents typically comprise amorphous nanoparticles. Additionally, there are disclosures of nanoparticulate materials comprising carbonate in the crystalline calcite and vaterite forms.

The basicity of the detergents may also be expressed as a total base number (TBN). A total base number is the amount of acid needed to neutralize all of the basicity of the overbased material. The TBN may be measured using ASTM standard D2896 or an equivalent procedure. The detergent may have a low TBN (i.e. a TBN of less than 50), a medium TBN (i.e. a TBN of 50 to 150) or a high TBN (i.e. a TBN of greater than 150, such as 150-500). In this invention, Basicity Index and Degree of Carbonation may be used. Basicity Index is the molar ratio of total base soap in the overbased detergent. Degree of Carbonation is the percentage of carbonate present in the overbased present in the overbased detergent expressed as a mole percentage relative to the total excess base in the detergent.

Overbased metal hydrocarbyl-substituted hydroxybenzoates can be prepared by any of the techniques employed in the art. A general method is as follows:

1. Neutralisation of hydrocarbyl-substituted hydroxybenzoic acid with a molar excess of metallic base to produce a slightly overbased metal hydrocarbyl-substituted hydroxybenzoate complex, in a solvent mixture consisting of a volatile hydrocarbon, an alcohol and water;
2. Carbonation to produce colloidally-dispersed metal carbonate followed by a post-reaction period;
3. Removal of residual solids that are not colloidally dispersed; and
4. Stripping to remove process solvents.

Overbased metal hydrocarbyl-substituted hydroxybenzoates can be made by either a batch or a continuous overbasing process.

Metal base (e.g. metal hydroxide, metal oxide or metal alkoxide), preferably lime (calcium hydroxide), may be charged in one or more stages. The charges may be equal or may differ, as may the carbon dioxide charges which follow them. When adding a further calcium hydroxide charge, the carbon dioxide treatment of the previous stage need not be complete. As carbonation proceeds, dissolved hydroxide is converted into colloidal carbonate particles dispersed in the mixture of volatile hydrocarbon solvent and non-volatile hydrocarbon oil.

Carbonation may be effected in one or more stages over a range of temperatures up to the reflux temperature of the alcohol promoters. Addition temperatures may be similar, or different, or may vary during each addition stage. Phases in which temperatures are raised, and optionally then reduced, may precede further carbonation steps.

The volatile hydrocarbon solvent of the reaction mixture is preferably a normally liquid aromatic hydrocarbon having a boiling point not greater than about 150° C. Aromatic hydrocarbons have been found to offer certain benefits, e.g. improved filtration rates, and examples of suitable solvents are toluene, xylene, and ethyl benzene.

The alkanol is preferably methanol although other alcohols such as ethanol can be used. Correct choice of the ratio of alkanol to hydrocarbon solvents, and the water content of the initial reaction mixture, are important to obtain the desired product.

Oil may be added to the reaction mixture; if so, suitable oils include hydrocarbon oils, particularly those of mineral origin. Oils which have viscosities of 15 to 30 mm<sup>2</sup>/sec at 38° C. are very suitable.

After the final treatment with carbon dioxide, the reaction mixture is typically heated to an elevated temperature, e.g. above 130° C., to remove volatile materials (water and any remaining alkanol and hydrocarbon solvent). When the synthesis is complete, the raw product is hazy because of the presence of suspended sediments. It is clarified by, for example, filtration or centrifugation. These measures may be used before, or at an intermediate point, or after solvent removal.

The products are generally used as an oil solution. If the reaction mixture contains insufficient oil to retain an oil solution after removal of the volatiles, further oil should be added. This may occur before, or at an intermediate point, or after solvent removal.

In this invention, (B) may have:

- (B1) a basicity index of less than two and a degree of carbonation of 80% or greater; or
- (B2) a basicity index of two or greater and a degree of carbonation of 80% or greater; or
- (B3) a basicity index of two or greater and a degree of carbonation of less than 80%; or
- (B4) a basicity index less than of two and a degree of carbonation of less 80%.

The treat rate of additive (A), or additives (A) and (B), contained in the lubricating oil composition may for example be in the range of 1 to 25, preferably 2 to 20, more preferably 5 to 18, mass %, subject to any limitations indicated herein. Co-Additives

The lubricating oil composition of the invention may comprise further additives, different from and additional to (A) and (B) (if (B) is used). Such additional additives may, for example include ashless dispersants, other metal detergents, anti-wear agents such as zinc dihydrocarbyl dithiophosphates, anti-oxidants and demulsifiers.

It may be desirable, although not essential, to prepare one or more additive packages or concentrates comprising the additives, whereby additives (A) and (B) (if (B) is required) can be added simultaneously to the base oil to form the lubricating oil composition. Dissolution of the additive package(s) into the lubricating oil may be facilitated by solvents and by mixing accompanied with mild heating, but this is not essential. The additive package(s) will typically be formulated to contain the additive(s) in proper amounts to provide the desired concentration, and/or to carry out the intended function in the final formulation when the additive package(s) is/are combined with a predetermined amount of base lubricant. Thus, additives (A) and (B) (if (B) is required), in accordance with the present invention, may be admixed with small amounts of base oil or other compatible solvents together with other desirable additives to form additive packages containing active ingredients in an amount, based on the additive package, of for example, from 2.5 to 90, preferably from 5 to 75, most preferably from 8 to 60, mass % of additives in the appropriate proportions, the remainder being base oil.

The final formulations as a trunk piston engine oil may typically contain 3 or 5 to 30, preferably 10 to 28, more preferably 12 to 24, mass % of the additive package(s), the remainder being base oil. Preferably, the trunk piston engine oil has a compositional TBN (using ASTM D2896) of 20 to 60, such 25 to 55. When (B) is present, the relative mass:mass proportions of (A) to (B) may, for example, be in the range of 10:1 to 1:10, such as 5:1 to 1:5, such as 3:1 to 1:3.

## EXAMPLES

The present invention is illustrated by but in no way limited to the following examples.

## Components

The following components were used:

Component (A1): 3-pentadecylphenol (ex Sigma Aldrich);  
Component (A2): distilled technical CNSL or "cardanol" (ex Palmer International);

Component (B): a calcium, salicylate detergent having a TBN of 350 (basicity index of two or greater; a degree of carbonation of 80% or greater) and containing 6 mass % of alkylphenol;

Base oil II: an API Group II base oil known as CHEV600R  
HFO: a heavy fuel oil, ISO-F-RMK 380

## Lubricants

Selections of the above components were blended to give a range of trunk piston marine engine lubricants. Some of the lubricants are examples of the invention; others are reference examples for comparison purposes. The compositions of the lubricants tested when each contained HFO are shown in the tables below under the "Results" heading.

## Testing

## Light Scattering

Test lubricants were evaluated for asphaltene dispersancy using light scattering according to the Focused Beam Reflectance Method ("FBRM"), which predicts asphaltene agglomeration and hence 'black sludge' formation.

The FBRM test method was disclosed at the 7<sup>th</sup> International Symposium on Marine Engineering, Tokyo, 24<sup>th</sup> 28<sup>th</sup> Oct. 2005, and was published in 'The Benefits of Salicylate Detergents in TPEO Applications with a Variety of Base Stocks', in the Conference Proceedings. Further details were disclosed at the CIMAC Congress, Vienna, 21<sup>st</sup>-24<sup>th</sup> May 2007 and published in "Meeting the Challenge of New Base Fluids for the Lubrication of Medium Speed Marine Engines—An Additive Approach" in the Congress Proceedings. In the latter paper it is disclosed that by using the FBRM method it is possible to obtain quantitative results for asphaltene dispersancy that predict performance for lubricant systems based on basestocks containing greater than or less than 90% saturates, and greater than or less than 0.03% sulphur. The predictions of relative performance obtained from FBRM were confirmed by engine tests in marine diesel engines.

The FBRM probe contains fibre optic cables through which laser light travels to reach the probe tip. At the tip, an optic focuses the laser light to a small spot. The optic is rotated so that the focussed beam scans a circular path between the window of the probe and the sample. As particles flow past the window they intersect the scanning path, giving backscattered light from the individual particles.

The scanning laser beam travels much faster than the particles; this means that the particles are effectively stationary. As the focussed beam reaches one edge of the particle there is an increase in the amount of backscattered light; the amount will decrease when the focussed beam reaches the other edge of the particle.

The instrument measures the time of the increased backscatter. The time period of backscatter from one particle is multiplied by the scan speed and the result is a distance or chord length. A chord length is a straight line between any two points on the edge of a particle. This is represented as a chord length distribution, a graph of numbers of chord lengths (particles) measured as a function of the chord length dimensions in microns. As the measurements are performed in real time the statistics of a distribution can be calculated and tracked. FBRM typically measures tens of thousands of chords per second, resulting in a robust number-by-chord length distribution. The method gives an absolute measure of the particle size distribution of the asphaltene particles.

The Focused beam Reflectance Probe (FBRM), model Lasentec D600L, was supplied by Mettler Toledo, Leicester, UK. The instrument was used in a configuration to give a particle size resolution of 1 µm to 1 mm. Data from FBRM can be presented in several ways. Studies have suggested that the average counts per second can be used as a quantitative determination of asphaltene dispersancy. This value is a function of both the average size and level of agglomerate. In this application, the average count rate (over the entire size range) was monitored using a measurement time of 1 second per sample.

The test lubricant formulations were heated to 60° C. and stirred at 400 rpm; when the temperature reached 60° C. the FBRM probe was inserted into the sample and measurements made for 15 minutes. An aliquot of heavy fuel oil (10% w/w) was introduced into the lubricant formulation under stirring using a four blade stirrer (at 400 rpm). A value for the average counts per second was taken when the count rate had reached an equilibrium value (typically overnight).

## 20 Results

## Light Scattering

The results of the FBRM tests are summarized in TABLE 1 below. In TABLE 1, phenols A1 and A2 were each blended separately with overbased Ca salicylate (B).

The base oil was Base oil II.

Wt. values are mass % a.i. The results are particle count values. By way of comparison, values for the salicylate alone are also indicated.

TABLE 1

|    | Identity of Phenol            |                            |                  |
|----|-------------------------------|----------------------------|------------------|
|    | % Phenol A/<br>% Salicylate B | A1<br>(3-pentadecylphenol) | A2<br>(cardanol) |
| 35 | 0/0                           | 27,920                     | —                |
|    | 3.84/0                        | 33,027*                    | 37,933*          |
|    | 7.68/0                        | 13,980*                    | —                |
|    | 0/5.73                        | 13,123                     | 13,278           |
| 40 | 1.92/5.73                     | 2,467*                     | 11,697*          |
|    | 3.84/5.73                     | 28*                        | 5,430*           |
|    | 7.68/5.73                     | 13*                        | 18*              |
|    | 11.52/5.73                    | 14*                        | 15*              |

\*= inventive examples

The results below the bar show that, in combination with the salicylate, A1 (a phenol of the invention) gives performance benefits and that A2 (also a phenol of the invention) also exhibits performance benefits. Also, results above the bar show that A1 without the salicylate is effective.

The invention claimed is:

1. A trunk piston marine engine lubricating oil composition for improving asphaltene handling in use thereof in operation of the engine when fuelled by a heavy fuel oil, which composition comprises or is made by admixing an oil of lubricating viscosity, in a major amount, and, in a minor amount:

(A) one or more oil-soluble phenolic compounds, comprising one or more of 3-pentadecylphenol and 5-pentadecylresorcinol, wherein 50 or more mass % of said one or more oil soluble phenolic compounds is 3-pentadecylphenol, where the pentadecyl group is linear and is attached to the aromatic ring at its first carbon atom, provided that, in the absence of an hydroxybenzoate detergent, the mass percentage of the phenolic compound is 4 or more.

2. The composition as claimed in claim 1 further including in a minor amount:

**11**

- (B) an overbased metal hydrocarbyl-substituted hydroxybenzoate detergent.
3. The composition as claimed in claim 2 where (B) has
- (B1) a basicity index of less than two and a degree of carbonation of 80% or greater; or
- (B2) a basicity index of two or greater and a degree of carbonation of 80% or greater; or
- (B3) a basicity index of two or greater and a degree of carbonation of less than 80%; or
- (B4) a basicity index of less than two and a degree of carbonation of less 80%,

where degree of carbonation is the percentage of carbonate present in the overbased metal hydrocarbyl-substituted hydroxybenzoate detergent expressed as a mole percentage relative to the total excess base in the detergent.

4. The composition as claimed in claim 2 where the metal in (B) is calcium.

5. The composition as claimed in claim 2 where the hydrocarbyl-substituted hydroxybenzoate in (B) is a salicylate.

6. The composition as claimed in claim 1 where the oil of lubricating viscosity contains 50 mass % or more of a basestock containing greater than or equal to 90% saturates and less than or equal to 0.03% sulphur or a mixture thereof.

**12**

7. The composition as claimed in claim 6 where the basestock containing greater than or equal to 90% saturates and less than or equal to 0.03% sulphur is a Group II basestock.

8. The composition as claimed in claim 1 having a TBN of 5 to 60.

9. A method of operating a trunk piston engine medium-speed compression-ignited marine engine comprising

(i) fueling the engine with a heavy fuel oil; and

(ii) lubricating the crankcase of the engine with a composition as defined in claim 1.

10. A method of dispersing asphaltenes in a trunk piston marine lubricating oil composition during its lubrication of surfaces of the combustion chamber of a marine-speed compression-ignited marine engine and operation of the engine, which method comprises

- (i) providing a composition as defined in claim 1;
- (ii) providing the composition in the combustion chamber;
- (iii) providing heavy fuel oil in the combustion chamber; and
- (iv) combusting the heavy fuel oil in the combustion chamber.

\* \* \* \* \*